

# UNITED STATES PATENT OFFICE.

MAJOR E. HOLMES, OF LAKEWOOD, OHIO, ASSIGNOR, BY MESNE ASSIGNMENTS, TO  
NATIONAL CARBON COMPANY, INC., A CORPORATION OF NEW YORK.

## BATTERY-DEPOLARIZER

1,259,099.

Specification of Letters Patent. Patented Mar. 12, 1913.

No Drawing.

Application filed September 10, 1914. Serial No. 861,074.

To all whom it may concern:

Be it known that I, MAJOR E. HOLMES, a citizen of the United States, residing at Lakewood, in the county of Cuyahoga and State of Ohio, have invented a certain new and useful Improvement in Battery-Depolarizers, of which the following is a full, clear, and exact description.

My invention relates to depolarizers for electric batteries and is primarily adapted for that type of electric battery known as dry cells.

Dry cells have for a long time been constructed with pyrolusite as depolarizer. This material is much too dense for efficient action, and does not pack into the dry cell container as readily as desired. Pyrolusite also contains impurities that not only occupy space that should contain depolarizer, but also injuriously affect the cell's action. It is not sufficiently active, chemically, to react with all the hydrogen when the cell is subjected to severe service, as when used in flashlight batteries. It is the object of my invention to treat the natural mineral pyrolusite so as to overcome the above difficulties. Before incorporating pyrolusite in a dry cell containing the usual carbon electrode and zinc can, I subject it to the action of sodium hydroxid, or other hydroxid, under pressure. Below 175° the rate of the reaction is slow, but if pyrolusite is heated to this temperature at normal atmospheric pressure it is reduced to a lower oxid, namely  $Mn_3O_4$ . Since this lower oxid is not reduced by hydrogen at ordinary temperatures, it is of no value as a depolarizer, and the above treatment must take place under sufficient pressure to prevent the reduction of the pyrolusite. It has been found that the most suitable temperature for bringing about the reaction is approximately 188° C.

When a solution of sodium hydroxid is heated with air and pyrolusite under pressure, the latter is hydrated. While this takes place in one continuous reaction, it nevertheless probably takes place in two stages as shown by the following equations:



The material can also be made by mixing powdered sodium hydroxid, or other hydroxid, with powdered pyrolusite and some

oxidizing agent such as a chlorate, perchlorate, nitrate, etc., and heating, preferably until fusion takes place. This produces sodium manganate which is then converted into the hydrated peroxid by crushing and treating with steam. It will be apparent that the modified process produces the desired result in two entirely separate steps. The fusion of the hydroxid with the pyrolusite produces the reaction set forth in the first equation previously given, while the treatment of the sodium manganate, with steam produces the reaction set forth in the second equation. The modified process is claimed in my divisional application filed September 15, 1916, Serial No. 120,273.

The pyrolusite, after being treated in either way, is transformed into a very fine powder of less density and higher compressibility than the original material. This not only enables it to be better tamped in the zinc can, but also permits its separation from the impurities in the pyrolusite which have not been acted upon by the hydroxid solution. These impurities are not in such a fine state of division and therefore can be separated from the manganese peroxid by the use of sieves of proper mesh.

Pyrolusite, when acted upon by an alkaline solution as described, has much greater activity as a depolarizer, and hence is preferable to the native pyrolusite for dry cell work.

Another distinct advantage in the treated product is in its increased absorptive power. The treated material when incorporated in a dry cell as the depolarizer therefore absorbs more electrolyte solution than the natural pyrolusite, which not only increases the energy output but also prevents the premature drying out of the cell.

The hydrated material has a slight tendency to react with the zinc chloride in a dry cell mix to form hydrochloric acid which attacks the zinc regardless of whether the cell is being used or not. The amount of the acid formed is of course small and it is not objectionable if cells are put into use on heavy service within a reasonable time after being made, but a long shelf life is of prime importance in certain other uses, and to prevent this reaction I dehydrate the product. This may be done by calcining it to drive off the water of hydration, as described in my co-pending application filed December 21, 110

1912, Serial No. 732,615, which has become Patent No. 1,184,854.

The calcined product has the same advantageous physical properties as before calcination, such as fine state of division, greater compressibility and increased absorptive power, etc. These physical characteristics, however, not only have their physical effect when the depolarizer is used in a dry cell mix, but also increase the chemical activity of the material. Such effect of physical state on chemical activity is well known in other arts. For instance, coal at ordinary temperatures does not oxidize, but when it is ground into fine dust particles its oxidation is so instantaneous as to cause violent explosions of not infrequent occurrence in coal mines. Pyrolusite in an analogous way has undergone an advantageous change in spite of the fact that the calcination probably brings it back into its original chemical form.

Both the hydrated and dehydrated pyro-

lusite, that is dehydrated hydrated-pyrolusite, have their particular advantages in certain cases, and either form will be used depending upon the particular use to which the dry cell containing it is put.

I am aware that artificial hydrated manganese peroxid has been made by treating certain manganese salts with various reagents, but the product obtained by my invention is not the same as such artificial product, as various tests show.

Having described my invention, what I claim is:

The process of purifying pyrolusite and increasing its depolarizing action when used in electric batteries which consists in heating it in a hydroxid solution under pressure.

In testimony whereof, I hereunto affix my signature in the presence of witnesses.

MAJOR E. HOLMES.

Witnesses:

H. G. GROVER,  
D. C. REED.